

Sept. 4, 1956

M. B. CHRISTIAN ET AL

2,761,804

METHOD OF MAKING PAPER-COVERED WOOD VENEER SHOOTS

Filed May 8, 1953



1

2,761,804

**METHOD OF MAKING PAPER-COVERED WOOD VENEER SHOOKS**

Moss B. Christian and Horace F. Ladd, Tallulah, La., assignors to Chicago Mill and Lumber Company, Chicago, Ill., a corporation of Delaware

Application May 8, 1953, Serial No. 353,874

5 Claims. (Cl. 154—118)

This invention relates to paper-covered box blanks or shooks and includes method and apparatus for producing the same. Particularly, this invention relates to a wrap-around, paper-covered folding box blank composed of a row of transversely spaced wood veneer pieces with gaps therebetween and having paper covers adhesively united to the wood veneer pieces and extending across the gaps for providing bending hinges connecting the veneer pieces.

In accordance with this invention green or undried wood veneer with a moisture content of 30 per cent or more and having the cells thereof in wet swollen condition is cut to size to provide panel sections for the bottom, sides and top lids of a box. The cut veneer pieces are adhesively coated and deposited on a sheet of tough, unsized kraft paper. This kraft paper is preferably coated with wax and a mold preventative. The cut veneer pieces have the grain thereof extending transversely across the width of the kraft sheet and project beyond the edges of the paper. Two sheets of kraft paper are then deposited on the coated veneer pieces and another set of glue-coated veneer pieces is deposited on the topmost of the two sheets. In this manner, a stack of veneer pieces covered on both sides with kraft paper is built up and this stack is then pressed by means of clamps or the like to firmly hold the paper against the wood and create an initial bond with the adhesive. The apparatus of this invention includes a base or platform with upright spacer bars receiving the wood veneer pieces therebetween to automatically align the pieces on the kraft paper and provide gaps between the pieces of the desired width. These gaps accommodate bending of the paper between adjacent veneer pieces into right angular relation for forming the wrap-around box or shook. The glue is set sufficiently in the stack to form a bond before the wood is dried below 30 per cent moisture content. The paper covers are thus firmly bonded to the wood to hold it against shrinkage. The bonded assemblies are then passed between hot rolls to dry the wood and further set the glue. The dried assemblies will have a moisture content of from 6 to 12 per cent but the wood will be in the expanded open cellular condition of wet wood. The dried and completely set assemblies are then trimmed to size and the ends of the wood pieces projecting beyond the paper covers are cut off.

It is then an object of this invention to provide a paper-covered wrap-around carton blank having a wood center with the wood pieces therein separated from each other to provide spaces for bending the paper into carton or box shape.

A specific object of this invention is to provide a paper-covered expanded wood veneer shook with the paper covers forming the sole joint between the veneer pieces to create free-folding corner joints.

Another object of this invention is to provide a wrap-around folding box blank composed of a row of five spaced wood veneer pieces having paper covers adhesively united to both faces of the pieces and with each piece

2

having a moisture content of from 6 to 12 per cent but held by the paper covers in the open expanded cellular network of wood having a moisture content of at least 30 per cent.

5 A still further object of this invention is to provide a wrap-around box shook composed of paper-covered wood veneer pieces to form the sides, the bottom, and the top lids of a box.

10 A further object of this invention is to provide a paper-covered wood veneer assembly adapted to be wrapped around wood end pieces to form a finished carton or box.

15 A still further object of this invention is to provide apparatus for forming paper-covered wood veneer shooks which includes upright dividers to hold the veneer pieces in properly aligned and spaced relationship.

20 A still further object of the invention is to provide a method for producing paper-covered wood veneer box blanks by stacking wood veneer pieces between dividers and by incorporating paper sheets between the veneer pieces in each stack.

Other and further objects of this invention will be apparent to those skilled in the art from the following detailed description of the annexed sheet of drawings 25 which, by way of a preferred example, illustrates the product of this invention and the apparatus for producing the product.

On the drawings:

30 Figure 1 is an isometric view of a paper-covered wood veneer shook according to this invention.

Figure 2 is an isometric view of a finished box made from the shook of Figure 1.

Figure 3 is a plan view of the wrap-around shook of this invention.

35 Figure 4 is a longitudinal cross-sectional view taken along the line IV—IV of Figure 3.

Figure 5 is a plan view of apparatus for forming the shooks of this invention and illustrating the manner in which the paper sheet and the wood veneer pieces are 40 inserted in the apparatus.

Figure 6 is a side elevational view of the apparatus of Figure 5 and illustrating a stack of veneer sheets and wood veneer pieces therein.

45 Figure 7 is a plan view of the assembly formed in the stack of Figure 6 after it is removed from the stacking apparatus and illustrating the projecting ends of the veneer pieces.

As shown on the drawings:

The shook 10 of Figure 1 has a bottom 11, sides 12 and 13 in right angular relation and top lids 14 and 15. The bottom 11 has a single piece of plywood 16 extending throughout its length and width. The grain of the plywood piece 16 runs lengthwise of the shook. The sides 12 and 13 have similar plywood pieces 17 and 18 respectively. The lids 14 and 15 have narrower plywood pieces 19 and 20 respectively. An inside paper cover 21 and an outside paper cover 22 is adhesively bonded to the opposite faces of the plywood pieces 16 to 20 and extends between these pieces to form bending 60 hinges 23.

A finished box 10a shown in Figure 2, is formed from the shook 10 by securing the bottom, the sides and the top lids around the periphery of wood end pieces such as 24. Nails or other fasteners 25 are used to attach 65 the shook to the end pieces. As illustrated in Figure 2, the wood end 24 will have a square or rectangular configuration adapted to fit within the space at the end of the shook when the sides of the shook are positioned at right angular relation to the bottom and when the top lids are positioned in right angular relation to the sides. A rectangular box is thereby provided. The box

can be sealed by placing an adhesive tape 26 over the space between the top lids 14 and 15.

As illustrated in Figures 3 and 4, the shook 10 when laid out flatwise, has the bottom wood veneer piece 11 in the center thereof with the side pieces 12 and 13 on each side thereof and with the end lid 14 outside of the side piece 12 while the end lid 15 is outside of the side piece 13. The gaps 23 between the wood veneer pieces 16 to 20 forming the bottom, sides and end pieces, are sufficiently wide relative to the thickness of the wood veneer so that the adjacent wood veneer pieces can be bent into right angular relationship without rupturing the paper covers 21 and 22. As shown in Figure 4, adhesive bonds 26 and 27 unite the paper covers 21 and 22 to the wood veneer pieces and the adhesive forming these bonds extends into the pores of the wood and paper to create firm anchoring locks which hold the wood against shrinkage.

Suitable apparatus 28 for laying up the shook assemblies 10 is shown in Figures 5 and 6. This apparatus 28 includes a base or bottom 29 with upstanding divider bars 30 along each longitudinal edge thereof. These bars are arranged in transversely aligned pairs on the opposite longitudinal edges of the base, and are spaced longitudinally to provide therebetween chambers for snugly receiving the respective wood veneer pieces of the shook. The dividers are wide enough to form the desired gaps 23 between the veneer pieces.

The base 29 receives the bottom kraft paper sheet 22 thereon and the veneer pieces 16 to 20 are glue-coated on both faces and are laid between the respective dividers 30 to form the assembly shown in Figure 5. Alternately, the top face of the kraft sheet 22 can be glue-coated instead of the veneer pieces. Two kraft cover sheets 21 and 22 are then deposited on top of the veneer pieces between the dividers. As shown in Figure 6 the two kraft cover sheets 21 and 22 are in face-to-face relation so that the bottom sheet 21 will form the top cover for the bottom row of veneer pieces while the top sheet 22 will form the bottom cover sheet for the next row of veneer pieces in the stack. The successive assemblies of paper sheets and wood veneer pieces is continued until a stack of desired height is formed in the apparatus 28. As shown, the kraft sheets are narrower than the wood veneer pieces so as to lie inside of the dividers while the veneer pieces project between the dividers to be held thereby in the proper spaced relation. The grain of the veneer pieces extend transversely across the width of the apparatus and across the length of the kraft sheets 21 and 22.

As shown in Figure 6, when a stack of desired height is provided in the apparatus 28, clamps 31 or other loading means are utilized to press the stack and firmly force the paper and wood into intimate contact. The pressing is done without heat and is maintained until an initial glue bond is formed which will hold the wet wood against shrinkage during subsequent drying operations. The paper sheets and the glue bonds in preventing shrinkage of the wood during the drying operation will actually hold the wood in an open expanded cellular condition of substantially the same size as the wet swollen wood without, however, retaining the moisture in the wood cells. Alkaline soya-bean glue is a desired bonding adhesive although other types of cold-setting adhesives can be used. After the glue bonds have been formed on the wet wood the clamps or other loading means are removed and the successive assemblies are removed from the apparatus 28. As shown in Figure 7, the shook assemblies 10 in their untrimmed state, have the ends of the plywood pieces projecting beyond the sides of the kraft paper and these projecting ends are trimmed off to provide the finished shook of Figures 1 to 4. Prior to trimming it is desirable to hot roll the assemblies in a drier to dry the wood to a moisture content of between 6 and 12 per cent. The hot rolling further sets the glue bonds and presses the paper into intimate contact with the wood.

From the above descriptions it will, therefore, be understood that this invention provides a wrap-around paper-covered wood veneer shook adapted to be easily converted into a finished box or carton with the use of end walls. These end walls are preferably made of wood but can be formed of any other suitable box or crate material. The shooks of this invention are strong, durable and light in weight. The single thickness veneer pieces constituting the shooks coat with the tough kraft paper through the media of a firm glue bond which is set before the wood is dried so that the wood is held in its open cellular condition of wet wood while only retaining from 6 to 12 per cent moisture. This open cellular wood is free from splits and cracks which ordinarily occur in the drying of veneer and is more supple than ordinary dried veneer.

We claim as our invention:

1. The method of making paper-covered wood veneer shooks which comprises stacking wood veneer pieces between dividers to form rows of pieces in spaced relation, covering each row with paper sheets of a width accommodated between said dividers and of a length equal to the combined widths of said veneer pieces plus the spaces therebetween, and adhesively bonding the paper sheets to the wood pieces.

2. The method of forming folding box blanks composed of paper-covered wood veneer pieces which comprises laying a row of wood veneer pieces between paper covers with each piece spaced from an adjacent piece and projecting beyond the edges of the paper covers, adhesively uniting the pieces in each row to the adjacent paper covers and trimming off the projecting margins of said veneer pieces to the edges of said paper covers.

3. The method of making paper-covered folding box blanks composed of wood veneer pieces covered by paper sheets forming hinges between the wood veneer pieces which comprises depositing a paper sheet centrally between longitudinally spaced upright dividers on a base, depositing wet glue-coated wood veneer pieces transversely on the paper sheet extending between the dividers beyond the sides of the sheet to be spaced apart for forming gaps therebetween, depositing two sheets of paper on the thus-formed row of wood veneer pieces, depositing another row of glue-coated wood veneer pieces on top of the uppermost sheet of said two sheets of paper and extending between the dividers repeating the alternate deposition of rows of wood veneer pieces and two sheets of paper to form a stack of desired height, pressing the stack to intimately unite the paper and wood, allowing the adhesive to set in the pressed stack without drying the wood to its shrinkage point, releasing the pressure, removing the resulting blank assemblies from the stack, drying the assemblies to a moisture content between 6 to 12 per cent while the paper holds the wood against shrinkage, and trimming off the ends of the wood veneer pieces projecting beyond the sides of the sheets.

4. The method of forming folding paper-covered wood shooks which comprises alternately stacking wood veneer pieces and paper covers to form rows of wood veneer pieces in spaced parallel relation and projecting beyond the paper covers, pressing the stack to set the adhesive, drying the assembly, and trimming off the projecting wood pieces.

5. The method of making folding box shooks which comprises forming alternate layers of paper covers and rows of wood veneer pieces in spaced parallel relation, said wood veneer pieces being in wet swollen condition with a moisture content of over 30 per cent, adhesively uniting the rows of wood veneer pieces to the adjacent paper covers, thereafter drying the wood to a moisture content between 6 to 12 per cent and holding the wood against shrinkage by said paper covers and glue bonds to maintain the wood in its wet swollen condition.

## References Cited in the file of this patent

## UNITED STATES PATENTS

|           |                |               |
|-----------|----------------|---------------|
| 1,217,852 | Walker         | Feb. 27, 1917 |
| 1,864,812 | Elmendorf      | June 28, 1932 |
| 1,875,056 | Loetscher      | Aug. 30, 1932 |
| 1,997,344 | Randall et al. | Apr. 9, 1935  |

|              |               |
|--------------|---------------|
| Duffy et al. | July 18, 1944 |
| Kantzler     | Jan. 27, 1953 |
| Elmendorf    | Mar. 10, 1953 |
| Elmendorf    | Nov. 9, 1954  |
| Elmendorf    | Nov. 9, 1954  |
| Elmendorf    | Oct. 4, 1955  |